

Nov. 22, 1960

E. E. BRYANT ET AL

2,961,337

METHOD OF METAL PREPARATION FOR PORCELAIN ENAMELING

Filed Oct. 8, 1958



*Mayer, Baldwin, Doran & Young*  
ATTORNEYS

1

2,961,337

**METHOD OF METAL PREPARATION FOR  
PORCELAIN ENAMELING**

Eugene E. Bryant, Cleveland, and Vaylord R. Luster, Medina, Ohio, assignors to Ferro Corporation, Cleveland, Ohio, a corporation of Ohio

Filed Oct. 8, 1958, Ser. No. 765,959

16 Claims. (Cl. 117—50)

This invention relates generally to decorative and protective coatings for application to steel and its alloys, and particularly to a method of preparing ferrous base metal to receive a single porcelain finish coat directly, without recourse to an intermediate ground or base coat.

Heretofore, steel preparation methods devised for direct application of vitreous enamel coatings to steel and its alloys have comprised generally the following steps: (1) A chemical or abrasive system for cleaning the steel of grease and organic matter. (2) One or more acid treatments to etch the ferrous work piece for improved adherence of the enamel and for uniform deposition of nickel in step three (3) which follows. The acid etch has also been effected by substituting an abrasive system for the acid treatment consisting generally of a sand or shot blasting operation. (3) A nickel "flash" or deposition either by an ion exchange method or electroless nickel deposition whereby a thin coating of metallic nickel is deposited, or plated onto the relatively clean and etched work piece, in an acid solution of pH in the range of 3.0 to 6.0. (4) Neutralizer bath of alkaline solution to prevent further oxidation caused by acidic residues and (5) drying. The importance of the nickel deposition step noted above is well known.

Utilizing the above noted sequence of steps, slight traces of organic greases and foreign matter acquired in milling of the steel, in transit, and fabricating the piece were not completely removed by the cleaning methods previously used, nor in subsequent acid treatment operations, so that such retained traces of organic matter, when subjected to the high temperatures of fusion of the vitreous enamel cover coats in the range of 1350° to 1500° F., volatilize and tend to give rise to pits and blisters in the direct-on cover coat. These pits and blisters form surface blemishes in the finished piece. It being clearly understood by one skilled in the art of course that the use of less viscous and more flexible intermediate ground coats prior to the application of the cover coat would eliminate the problem of defects, but the use of such intermediate ground coat is undesirable because of the need for an additional application, drying and firing operation plus the additional material required.

The nature of the surface of the steel and ferrous alloys is important in its preparation for direct-on application of cover coats. The surface should be uniform for good results. However, the surface of said ferrous alloys varies from mill to mill and from lot to lot produced in the same mill sufficiently to cause a variation in the rate of attack of acid pickling solutions resulting in a consequential variation in the degree of etch effected by the acid resulting in a consequential variation in the rate of deposition of nickel per unit area to the steel surface so that the critical limits of nickel deposition for a given operation tend to vary sufficiently to adversely affect the surface and adherence qualities of the finished enameled coating. This results in time-consuming delays while the temperature, pH and length of time of immersion of the

2

work piece in the acid and nickel solutions are readjusted to each lot of steel to compensate for variations in surface structure, in order to achieve a consistent degree of etch and deposition of nickel on the finished work piece

5 prior to enameling.

Thus we have found that by utilizing a physical heat treatment step in conjunction with any of the previously used steel preparation methods the variable "skin" of the ferrous alloy can be quickly and effectively removed.

10 Furthermore, all minute traces of foreign material usually insoluble to some extent in either the preceding cleaning or subsequent etching steps are removed by oxidizing both the "skin" plus traces of foreign matter so they can be uniformly and completely removed by subsequent etch

15 treatment.

In employing the heat treatment step, we have found that temperatures less than 1000° F. are incapable of producing the desired degree of oxidation, and temperatures above 1300° F. result in excessive and uneven oxidation.

20 For the most uniform removal of the "skin" and foreign matter from ferrous metal surfaces, temperatures in the range of 1100° F. to about 1200° F. are used, oxidizing the steel or ferrous alloy work piece the equivalent of from one to four grams of the ferrous base metal per

25 square foot.

It is an object of this invention to provide a method of preparing a ferrous work piece for a direct-on application of cover coat which is free of surface blemishes.

It is an object of this invention to provide a new method 30 of preparation of ferrous base metal for the direct application of vitreous cover coats in which the effect of work solutions on variable ferrous base metals is stabilized and an improved surface is produced for the application of direct-on vitreous enamel.

35 It is further the object of this invention to provide a method of porcelain enameling an article characterized by the elimination of conventional, intermediate ground coats in favor of a single, blemish-free finish coat applied directly on the base metal rather than over said intermediate coat.

40 It is a further object of this invention to provide a method for producing a superior enameled article by the application of a single finish coat direct to steel by depositing a highly uniform and even coating of nickel on its surface prior to application of the enamel cover coat.

In carrying out the invention, it is important that the oxidizing heat treatment be performed before the etching step.

45 While the use of a "grease burn" for the sole purpose 50 of removal of mill oil and shop lubricants from the ferrous work piece has been known for some time, such "grease burn" was in lieu of the cleaning operation rather than supplementary to it, and was performed at the elevated temperatures of 1500° to 1600° F. Furthermore, 55 such heat treatment, in lieu of a chemical or abrasive cleaning operation, had the effect of producing highly variable, uneven, and excessive oxidation of the work piece, said oxidation consisting of a complex mixture of insoluble iron soaps, partially oxidized organic compounds

60 and metal particles, which were carried over into the subsequent acid and/or nickel application steps, resulting in heavy contamination of these baths with resultant imperfections and blemishes in the finished cover coat, by virtue of the contaminants being picked up on the surface of the work pieces subsequently passed through said baths. On the other hand, the present invention utilizing the combination of oxidizing heat treatment at limited temperatures and an acid or abrasive etch produces an article having a light, thin, tight oxide layer

65 containing only traces of oxidized organic matter unremoved by the preceding cleaning operation, and consisting principally of the purer forms of oxides of iron 70

quickly and easily removed in the acid or abrasive etching treatments.

Our method, furthermore, gives rise to an oxidation of the variable surface "skin" of the work piece to a depth equivalent to one to four grams of iron per square foot, immediately under which thin layer of oxidation there lies a broadly planular surface unmarred by peaks and valleys caused by uneven oxidation, which planular surface is more highly conducive to the production of an evenly etched surface in the following etching step, which evenly etched surface, in turn, permits the even and uniform application of nickel over said evenly etched planular surface, which even application is so vital to the successful production of blemish-free enamel cover coats applied directly to steel.

#### STEEL SELECTION

While any grade of steel having less than 0.05% carbon generally may be utilized in conjunction with this invention, good results may be obtained by using a cold rolled steel, having the following metalloid analysis:

|             | Percent |
|-------------|---------|
| Carbon      | 0.03    |
| Manganese   | 0.05    |
| Phosphorous | 0.004   |
| Sulphur     | 0.025   |
| Silicon     | Trace   |

The gauge of the metal is limited only by the design of the work piece and ease of forming, and does not in any way alter the application of our process, except that the oxidizing heat treatment must be such that the article itself reaches the temperature indicated in the furnace, and then be permitted to "soak" for a period of about two minutes at indicated temperature.

The design of the article is of no particular importance, and since any one of innumerable designs and shapes have been successfully enameled, the subject article will be referred to as "work piece" throughout the specification and claims.

The work piece in accordance with the present invention is formed to a pre-designed shape and after forming, is processed by the following steps:

Alkaline cleaning, heat treatment, cooling, acid or abrasive etching, rinsing, nickel deposition, rinsing, drying, cover coat application, drying and firing.

The following example, in conjunction with the accompanying flow sheet drawing, illustrates the present invention:

#### Example

A 20 gage cold rolled steel sheet having an analysis as shown above, was formed into a panel and processed as indicated below.

I. *Cleaning operation.*—The work piece was submerged in an alkaline cleaning bath at a "rolling boil" at 212° F. for a minimum of 20 minutes. The cleaner was maintained at an active alkali content of 2% Na<sub>2</sub>O.

II. *Rinsing.*—The work piece was removed from the cleaner bath and submerged for from one to two minutes in clean, running water, maintained at a temperature of from 170° to 210° F.

III. *Secondary rinsing.*—The work piece was then immersed in a cold, clean water rinse at room temperature or less, for two minutes.

IV. *Drying.*—The alkaline cleaned and rinsed work piece was placed in a dryer, providing a clean circulating atmosphere, at a temperature between 300° to 375° F. It is understood that any suitable drying means may be used including continuous gas fired, oil fired, electrically heated or infra red dryers providing the work pieces are kept free of dirt or other foreign matter.

V. *Oxidation.*—The work piece was subjected to a temperature of 1200° F. for four minutes, two minutes being required to bring the piece to peak temperature, plus two

additional minutes at the indicated temperature in a commercial furnace having an oxidizing atmosphere.

VI. *Cooling.*—The work piece was removed from the furnace and permitted to cool to room temperature.

VII. *Acid pickle.*—The oxidized work piece was submerged in a phosphoric acid bath of 17±2% by volume, at a temperature of 125° F., for a time of six minutes, during which time all oxides were completely removed, and an even etch is achieved by the acid bath.

VIII. *Rinse.*—Work piece was submerged in clean running water of slightly acid pH (5.0 to 6.5) for a time of from 1½ to 2 minutes, said clean, running water at room temperature or below.

IX. *Nickel deposition.*—Using the well-known electroless method of application, such as described in U.S. Patent 2,532,283, the work piece was immersed in a bath containing 4.0 ounces±0.25 ounce per gallon of single nickel salts (Na<sub>2</sub>SO<sub>4</sub>·6H<sub>2</sub>O); 1.0±½ ounce sodium acetate per gallon; and 25 grams±5 grams sodium hypophosphite per gallon. This bath was maintained at a temperature of 87° F.±2° at a pH 3.5±0.3, for a time of 3½ minutes achieving a deposition of nickel by reduction on the work piece of approximately 0.065 gram of nickel per square foot of area exposed to the bath.

X. *Rinsing.*—The nickel-coated work piece was rinsed in clean, clear running water maintained at a temperature of 160° F.±20° F. for a time of 2 minutes±½ minute.

XI. *Drying.*—The work piece was placed in a suitable dryer having a clean, circulating atmosphere at a temperature of 300° F. to 400° F.

XII. *Enameling.*—After permitting to cool to room temperature, after drying, a titanium opacified cover coat of the composition listed below was applied so as to give a fired thickness of 0.005 inch±0.002 inch.

#### FRIT COMPOSITION

| Oxides:                                                                   | Parts by weight |
|---------------------------------------------------------------------------|-----------------|
| Li <sub>2</sub> O                                                         | 0.8             |
| Na <sub>2</sub> O                                                         | 11.0            |
| K <sub>2</sub> O                                                          | 6.0             |
| B <sub>2</sub> O <sub>3</sub>                                             | 16.2            |
| P <sub>2</sub> O <sub>5</sub>                                             | 2.5             |
| TiO <sub>2</sub>                                                          | 21.5            |
| SiO <sub>2</sub>                                                          | 42.0            |
|                                                                           | 100.0           |
| F <sub>2</sub> (percent replacing O <sub>2</sub> in above oxide analysis) | 4.5             |

#### 50 Mill addition:

|                                |     |
|--------------------------------|-----|
| Frit                           | 100 |
| Clay                           | 4   |
| K <sub>2</sub> CO <sub>3</sub> | ¼   |
| NaNO <sub>2</sub>              | ⅛   |
| Bentonite                      | ⅛   |
| Water                          | 42  |

After the enamel is applied to the work piece, it is dried and fired in an enameling furnace at a temperature of 1400° F. and for a time in the "hot zone" of the furnace to maintain the work piece at the indicated temperature for a period of 1½ minutes, for a total time of four minutes.

While the example set forth describes "submersion," of the work piece in various baths, this is meant to convey the idea of exposure of the work piece to the various baths described, either by actual immersion in a tank or vat containing the various solutions, or exposure of the work piece to the various solutions through a continuous spray machine wherein the solutions are maintained at the indicated temperatures and concentrations and the spray areas are of a length sufficient to subject the work piece to a given solution applied under pressurized spray for the required length of time.

It should be here pointed out also, that, although we

have used phosphoric acid and electroless nickel in the example, it is well known to those skilled in the art that any number of acids, such as hydrochloric and sulphuric, which will oxidize and etch steel will perform satisfactorily, as well as any method of applying the nickel coating which includes deposition by ion exchange and by reduction.

It is to be understood of course that variations may be made on this invention in order to meet different requirements without departing from the scope and intent of these specifications and the claims which follow.

Having thus described the invention, we claim:

1. In the process of preparing ferrous base metal for direct-on porcelain enameling in which the metal is subjected to a preliminary cleaning operation, the steps following said cleaning operation of heat-treating the ferrous base metal at a temperature of between about 1000° F. and 1300° F. long enough to oxidize from about one to four grams base metal per square foot of surface, and thereafter applying a porcelain enamel cover coat directly to the base metal.

2. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface and thereafter etching with phosphoric acid, neutralizing, drying and applying a finish coat of porcelain enamel directly to the metal.

3. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface and thereafter etching with sulphuric acid, neutralizing, drying, applying a cover coat of porcelain enamel directly to the metal and fusing the porcelain enamel thereon.

4. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface and thereafter etching with nitric acid, neutralizing, drying, applying a cover coat of porcelain enamel directly to the metal and fusing the porcelain enamel thereon.

5. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface thereafter etching with hydrochloric acid, neutralizing, drying, applying a cover coat of porcelain enamel directly to the metal and fusing the porcelain enamel thereon.

6. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface followed by an abrasive etching operation, followed by application of a porcelain enamel cover coat directly to the base metal, and fusing said porcelain enamel cover coat to the base metal.

7. In the process of preparing ferrous base metal for direct-on porcelain enameling in which the metal is subjected to a preliminary cleaning operation, the combination of heat-treating the cleaned base metal at a temperature of between 1100° F. and 1250° F. long enough

to oxidize from about one to four grams base metal per square foot of surface and thereafter etching with phosphoric acid, followed by application of a porcelain enamel cover coat directly to the base metal, and fusing said porcelain enamel cover coat to the base metal.

8. In the process of preparing ferrous base metal for direct-on porcelain enameling in which the metal is subjected to a preliminary cleaning operation, the combination of heat-treating the cleaned base metal at a temperature of between 1000° F. and 1300° F. long enough to oxidize from about one to four grams base metal per square foot of surface followed by a phosphoric acid etch, followed by a rinse, followed by nickel deposition of from 0.05 to 0.25 gram per square foot, followed by applying a porcelain enamel cover coat to the base metal.

9. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface followed by a sulphuric acid etch, followed by a rinse, followed by nickel deposition of from 0.05 to 0.25 gram per square foot, followed by applying a porcelain enamel cover coat to the base metal.

10. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface followed by a nitric acid etch, followed by a rinse, followed by nickel deposition of from 0.05 to 0.25 gram per square foot, followed by applying a porcelain enamel cover coat to the base metal.

11. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface followed by a hydrochloric acid etch, followed by a rinse, followed by nickel deposition of from 0.05 to 0.25 gram per square foot, followed by applying a porcelain enamel cover coat to the base metal.

12. In the process of preparing ferrous base metal for direct-on porcelain enameling in which the metal is subjected to a preliminary cleaning operation, the combination of heat-treating the cleaned base metal at a temperature of between about 1000° F. and 1300° F. long enough to oxidize from about one to four grams base metal per square foot of surface followed by an abrasive etching operation, followed by a rinse, followed by nickel deposition of from 0.05 to 0.25 gram per square foot, followed by applying a porcelain enamel cover coat to the base metal.

13. In the process of preparing ferrous base metal for direct-on porcelain enameling in which the metal is subjected to a preliminary cleaning operation, the combination of heat-treating the cleaned base metal at a temperature of between 1100° F. and 1250° F. long enough to oxidize from about one to four grams base metal per square foot of surface followed by a phosphoric acid etch, followed by a rinse, followed by nickel deposition of from 0.05 to 0.25 gram per square foot, followed by applying a porcelain enamel cover coat to the base metal.

14. In the process of preparing ferrous base metal for direct-on porcelain enameling in which the metal is subjected to a preliminary cleaning operation, the combination therewith of steps following said cleaning operation comprising heat treating the ferrous base metal at a temperature of between about 1000° F. and 1300° F. long enough to oxidize from about one to four grams of base metal per square foot of surface, removing the oxi-

dized metal layer coincidently with etching the underlying base metal surface in acid, depositing a layer of nickel on said etched surface at a concentration of from 0.05 to 0.25 gram per square foot, and thereafter applying a porcelain enamel cover coat directly to the base metal.

15. In the process of preparing ferrous base metal for direct-on porcelain enameling in which the metal is subjected to a preliminary cleaning operation, the combination therewith of steps following said cleaning operation comprising heat treating the ferrous base metal at a temperature of between about 1000° F. and 1300° F. long enough to oxidize from about one to four grams of base metal per square foot of surface, removing the oxidized metal layer coincidently with roughening the underlying base metal surface by an abrasive operation, depositing a layer of nickel on said etched surface at a concentration of from 0.05 to 0.25 gram per square foot, and thereafter applying a porcelain enamel cover coat directly to the base metal.

16. In the process of preparing ferrous base metal for 20

5  
10

direct-on porcelain enameling in which the metal is subjected to a preliminary cleaning operation, the combination therewith of steps following said cleaning operation comprising heat treating the ferrous base metal at a temperature of between about 1000° F. and 1300° F. long enough to oxidize from about one to four grams of base metal per square foot of surface, removing the oxidized metal layer coincidently with etching the underlying base metal surface, and thereafter applying a porcelain enamel cover coat directly to the base metal.

#### References Cited in the file of this patent

#### UNITED STATES PATENTS

|           |                 |               |
|-----------|-----------------|---------------|
| 2,099,340 | Kautz           | Nov. 16, 1937 |
| 2,206,597 | Canfield et al. | July 2, 1940  |
| 2,532,283 | Brenner et al.  | Dec. 5, 1950  |
| 2,581,310 | Sweo            | Jan. 1, 1952  |
| 2,812,270 | Alexander       | Nov. 5, 1957  |

UNITED STATES PATENT OFFICE  
CERTIFICATION OF CORRECTION

November 22, 1960

Patent No. 2,961,337

Eugene E. Bryant et al.

It is hereby certified that error appears in the above numbered patent requiring correction and that the said Letters Patent should read as corrected below.

In the drawing, the description of the nickel deposition bath, for "Na<sub>2</sub>SO<sub>4</sub>·6H<sub>2</sub>O" read -- NiSO<sub>4</sub>·6H<sub>2</sub>O --; in the printed specification, column 4, line 18, for "(Na<sub>2</sub>SO<sub>4</sub>·6H<sub>2</sub>O)" read -- (NiSO<sub>4</sub>·6H<sub>2</sub>O) --.

Signed and sealed this 20th day of June 1961.

(SEAL)

Attest:

ERNEST W. SWIDER

Attesting Officer

DAVID L. LADD  
Commissioner of Patents